

## UNITED STATES PATENT OFFICE

2,049,790

## REFRIGERATION

Harry M. Williams, Dayton, Ohio, assignor, by  
mesne assignments, to General Motors Corpora-  
tion, a corporation of Delaware

No Drawing. Application May 18, 1931,  
Serial No. 538,398

6 Claims. (Cl. 62—1)

This invention relates to refrigeration and more particularly to the sealing of refrigerating apparatus which is charged with certain fluorine compounds as refrigerants.

Heretofore when using fluorine containing substances, such as dichlorodifluoromethane or other halo-fluoro aliphatic derivatives of hydrocarbons as refrigerants in refrigerating apparatus, the sealing compound which has been used on gaskets of compressors, insulation windings of motors or other places in the refrigerating system has been dissolved in the refrigerant, so that the effectiveness of the seal has been destroyed. Objects of this invention include the provision of effective seals for these places which seals are not destroyed by the refrigerants being used in the refrigerating apparatus.

I have discovered that a mixture of vinyl acetate and vinyl chloride known commercially as Vinylite 80 provides such a seal, and that this mixture, when properly treated, is insoluble in certain halo-fluoro derivatives of the aliphatic hydrocarbons and particularly  $CF_2Cl_2$ . Thus this mixture overcomes difficulties heretofore experienced with this problem.

For example, the metal gaskets and the threads of fittings which are used on compressors of refrigerating systems and receivers, condensers and evaporators are coated or painted with a mixture of vinyl acetate and vinyl chloride, allowed to air dry, and the parts assembled together in the usual manner. Thereafter the compressors are heated during the process of enameling and drying for at least one hour at 200° F. in enameling ovens and a drying treatment of 10 hours at 225° F. in drying ovens. During such treatment the composition flows and is changed chemically so that it sets to a hard tough mass which is insoluble in the refrigerant.

Copper wire coils have been coated with this mixture and given a similar baking and drying treatment and it has been found that the coating is insoluble in such fluorine refrigerants.

The mixture of vinyl acetate and vinyl chloride may be mixed with a solvent such as toluene

by making a 35% solution of the mixture in toluene and such a solution forms an excellent lacquer-like material for application on the various parts of the refrigerating apparatus.

While the form of embodiment of the invention as herein disclosed, constitutes a preferred form, it is to be understood that other forms might be adopted, all coming within the scope of the claims which follow.

What is claimed is as follows:

1. The method of sealing refrigerating apparatus against the passage of organic refrigerants, which comprises coating a part of the apparatus exposed to the refrigerant with a mixture of vinyl acetate and vinyl chloride, and drying said mixture.

2. The method of sealing refrigerating apparatus against the passage of fluorine containing refrigerants, which comprises coating a part of the apparatus exposed to the refrigerant with a mixture of vinyl acetate and vinyl chloride and treating the apparatus by the application of heat sufficient to render said mixture insoluble in the refrigerant.

3. Refrigerating apparatus containing as a refrigerant a halogen derivative of an aliphatic hydrocarbon and having a separable joint in the refrigerant circuit of said apparatus treated with a mixture of vinyl acetate and vinyl chloride.

4. Refrigerating apparatus containing a halo-fluoro derivative of an aliphatic hydrocarbon and having a separable joint in the refrigerant circuit of said apparatus treated with a mixture of vinyl acetate and vinyl chloride.

5. Refrigerating apparatus charged with a fluorine containing refrigerant having a separable joint in the refrigerant circuit of said apparatus treated with a mixture of vinyl acetate and vinyl chloride.

6. Refrigerating apparatus containing an organic refrigerant having a separable joint in the refrigerant circuit of said apparatus treated with a mixture of vinyl acetate and vinyl chloride.

HARRY M. WILLIAMS.